



US012234198B2

(12) **United States Patent**  
**Mohler et al.**

(10) **Patent No.:** US 12,234,198 B2  
(45) **Date of Patent:** Feb. 25, 2025

(54) **PASSIVATED FUEL**(71) Applicant: **Spectre Enterprises, Inc.**, Melbourne, FL (US)(72) Inventors: **Timothy Mohler**, Melbourne, FL (US); **Daniel Yates**, Melbourne, FL (US)(73) Assignee: **Spectre Enterprises, Inc.**, Melbourne, FL (US)

(\* ) Notice: Subject to any disclaimer, the term of this patent is extended or adjusted under 35 U.S.C. 154(b) by 823 days.

(21) Appl. No.: **17/394,115**(22) Filed: **Aug. 4, 2021**(65) **Prior Publication Data**

US 2022/0041523 A1 Feb. 10, 2022

**Related U.S. Application Data**

(60) Provisional application No. 63/061,377, filed on Aug. 5, 2020.

(51) **Int. Cl.** **C06B 45/14** (2006.01)(52) **U.S. Cl.** CPC ..... **C06B 45/14** (2013.01)(58) **Field of Classification Search**

None

See application file for complete search history.

(56) **References Cited**

## U.S. PATENT DOCUMENTS

2,131,352 A 9/1938 Marsh  
2,239,123 A 4/1941 Stoneking

2,995,429 A 8/1961 Williams et al.  
2,995,431 A 8/1961 Bice  
3,122,884 A 3/1964 Grover et al.  
3,155,749 A 11/1964 Rossen et al.  
3,170,402 A 2/1965 Morton et al.  
3,275,259 A 9/1966 Plungulan  
3,382,117 A 5/1968 Cook  
(Continued)

## FOREIGN PATENT DOCUMENTS

GB 885409 A 12/1961  
GB 987332 A 3/1965  
(Continued)

## OTHER PUBLICATIONS

Jesse J. Sabatini, Amita V. Nagori, Gary Chen, Phillip Chu, Reddy Damavarapu, and Thomas M. Klapotke, High-Nitrogen-Based Pyrotechnics: Longer- and Brighter-Burning, Perchlo.

(Continued)

*Primary Examiner* — Aileen B Felton(74) *Attorney, Agent, or Firm* — Lang Patent Law LLC; William F. Lang, IV(57) **ABSTRACT**

A non-self-passivating fuel such as boron or magnesium is protected from exposure to oxygen sources by a self-passivating fuel layer such as aluminum or titanium. When the non-self-passivating fuel is utilized within a layered structure of alternating fuel and oxygen source layers, self-passivating fuel layers located between each non-self-passivating fuel layer and each oxygen source layer. The self-passivating fuel oxidizes until self-passivation is reached, protecting the non-self-passivating fuel from oxidation. Any of the non-self-passivating fuel which does not oxidize is available for use as fuel in any fuel-oxygen source reaction.

**11 Claims, 2 Drawing Sheets**

| (56)                  | References Cited |                       |                  |           |                  |                       |
|-----------------------|------------------|-----------------------|------------------|-----------|------------------|-----------------------|
| U.S. PATENT DOCUMENTS |                  |                       |                  |           |                  |                       |
| 3,668,872 A           | 6/1972           | Camp et al.           | 8,524,018 B2     | 9/2013    | Busky et al.     |                       |
| 3,711,344 A           | 1/1973           | Pierce                | 8,544,387 B2     | 10/2013   | Dahlberg         |                       |
| 3,715,248 A           | 2/1973           | Swotinsky et al.      | 8,591,676 B2     | 11/2013   | Coffey et al.    |                       |
| 3,725,516 A           | 4/1973           | Kaufman               | 8,641,842 B2     | 2/2014    | Hafner et al.    |                       |
| 3,794,545 A           | 2/1974           | Bertrand et al.       | 9,464,874 B1     | 10/2016   | Mohler et al.    |                       |
| 3,808,061 A           | 4/1974           | Pierce                | 9,709,366 B1     | 7/2017    | Mohler et al.    |                       |
| 3,896,731 A           | 7/1975           | Kilmer                | 9,816,792 B1     | 11/2017   | Mohler et al.    |                       |
| 3,896,865 A           | 7/1975           | Comfort et al.        | 10,254,090 B1    | 4/2019    | Mohler et al.    |                       |
| 3,905,846 A           | 9/1975           | Berta                 | 10,415,938 B2    | 9/2019    | Mohler et al.    |                       |
| 3,938,440 A           | 2/1976           | Dooley et al.         | 2006/0011276 A1  | 1/2006    | Grix et al.      |                       |
| 3,956,890 A           | 5/1976           | Davis                 | 2006/0278119 A1  | 12/2006   | Shilliday et al. |                       |
| 3,962,865 A           | 6/1976           | McCone, Jr.           | 2007/0169862 A1  | 7/2007    | Hugus et al.     |                       |
| 3,995,559 A           | 12/1976          | Bice et al.           | 2007/0272112 A1  | 11/2007   | Nielson et al.   |                       |
| 4,013,743 A           | 3/1977           | Blasche, Jr. et al.   | 2008/0047453 A1  | 2/2008    | Dahlberg         |                       |
| 4,115,999 A           | 9/1978           | Diebold               | 2008/0134924 A1  | 6/2008    | Sawka            |                       |
| 4,475,461 A           | 10/1984          | Durrell               | 2008/0202373 A1* | 8/2008    | Hugus            | F42B 12/44<br>102/506 |
| 4,615,270 A           | 10/1986          | Bell                  | 2009/0139422 A1  | 6/2009    | Mohler           |                       |
| 4,651,254 A           | 3/1987           | Brede et al.          | 2010/0032064 A1* | 2/2010    | Dreizin          | C06B 43/00<br>149/37  |
| 4,756,251 A           | 7/1988           | Hightower, Jr. et al. | 2010/0193093 A1  | 8/2010    | Coffey et al.    |                       |
| 4,823,699 A           | 4/1989           | Farinacci             | 2010/0251694 A1  | 10/2010   | Hugus et al.     |                       |
| 4,823,701 A           | 4/1989           | Wilhelm               | 2010/0282115 A1  | 11/2010   | Sheridan et al.  |                       |
| 4,875,948 A           | 10/1989          | Verneker              | 2011/0067789 A1  | 3/2011    | Grix et al.      |                       |
| 4,996,922 A           | 3/1991           | Halcomb               | 2011/0259230 A1  | 10/2011   | Sawka et al.     |                       |
| 5,030,301 A           | 7/1991           | Stout et al.          | 2011/0308416 A1  | 12/2011   | Bar et al.       |                       |
| 5,076,868 A           | 12/1991          | Doll et al.           | 2012/0103479 A1  | 5/2012    | Katzakian et al. |                       |
| 5,080,017 A           | 1/1992           | Asikainen             | 2012/0132096 A1  | 5/2012    | Chin et al.      |                       |
| 5,237,927 A           | 8/1993           | Gonzalez et al.       | 2013/0305950 A1  | 11/2013   | Coffman, II      |                       |
| 5,266,132 A           | 11/1993          | Danen et al.          | 2016/0102030 A1  | 4/2016    | Coffey et al.    |                       |
| 5,320,043 A           | 6/1994           | Andre et al.          | 2020/0232772 A1  | 7/2020    | Coffey et al.    |                       |
| 5,322,018 A           | 6/1994           | Hadden et al.         |                  |           |                  |                       |
| 5,363,768 A           | 11/1994          | Solberg et al.        |                  |           |                  |                       |
| 5,589,661 A           | 12/1996          | Menke et al.          |                  |           |                  |                       |
| 5,721,392 A           | 2/1998           | Chan et al.           |                  |           |                  |                       |
| 5,773,748 A           | 6/1998           | Makowiecki et al.     |                  |           |                  |                       |
| 5,801,325 A           | 9/1998           | Willer et al.         |                  |           |                  |                       |
| 5,817,970 A           | 10/1998          | Feierlein             |                  |           |                  |                       |
| 5,854,439 A           | 12/1998          | Almstrom et al.       |                  |           |                  |                       |
| 6,158,348 A           | 12/2000          | Campoli               |                  |           |                  |                       |
| 6,176,950 B1          | 1/2001           | Wood et al.           |                  |           |                  |                       |
| 6,183,569 B1          | 2/2001           | Mohler                |                  |           |                  |                       |
| 6,334,394 B1          | 1/2002           | Zimmermann et al.     |                  |           |                  |                       |
| 6,363,853 B1          | 4/2002           | Rohr                  |                  |           |                  |                       |
| 6,364,975 B1          | 4/2002           | Fleming et al.        |                  |           |                  |                       |
| 6,599,379 B2          | 7/2003           | Hiskey et al.         |                  |           |                  |                       |
| 6,679,960 B2          | 1/2004           | Jones                 |                  |           |                  |                       |
| 6,692,655 B1          | 2/2004           | Martins et al.        |                  |           |                  |                       |
| 6,712,917 B2          | 3/2004           | Gash et al.           |                  |           |                  |                       |
| 6,740,180 B1          | 5/2004           | Cesaroni              |                  |           |                  |                       |
| 6,805,832 B2          | 10/2004          | Mohler et al.         |                  |           |                  |                       |
| 6,843,868 B1          | 1/2005           | Fawls et al.          |                  |           |                  |                       |
| 6,962,112 B1          | 11/2005          | Kern                  |                  |           |                  |                       |
| 7,770,380 B2          | 8/2010           | Dulligan et al.       |                  |           |                  |                       |
| 7,886,668 B2          | 2/2011           | Hugus et al.          |                  |           |                  |                       |
| 7,896,988 B2          | 3/2011           | Mohler                |                  |           |                  |                       |
| 7,918,163 B2          | 4/2011           | Dahlberg              |                  |           |                  |                       |
| 7,955,451 B2          | 6/2011           | Hugus et al.          |                  |           |                  |                       |
| 7,958,823 B2          | 6/2011           | Sawka                 |                  |           |                  |                       |
| 7,998,290 B2          | 8/2011           | Sheridan et al.       |                  |           |                  |                       |
| 8,202,377 B2          | 6/2012           | Erickson et al.       |                  |           |                  |                       |
| 8,298,358 B1          | 8/2012           | Coffey et al.         |                  |           |                  |                       |
| 8,454,769 B2          | 6/2013           | Erickson et al.       |                  |           |                  |                       |
| 8,465,608 B1*         | 6/2013           | Coffey                | C06B 45/14       | 149/109.2 |                  |                       |

## FOREIGN PATENT DOCUMENTS

|    |                   |         |
|----|-------------------|---------|
| GB | 994184 A          | 6/1965  |
| WO | WO 2005/121055 A1 | 12/2005 |

## OTHER PUBLICATIONS

Marc Comet et al., Boron as Fuel for Ceramic Thermites (Abstract), Feb. 2014, <https://pubs.acs.org/doi/10.1021/ef500221p>.  
 Electroactive Polymers, Wikipedia, [https://en.wikipedia.org/wiki/Electroactive\\_polymer](https://en.wikipedia.org/wiki/Electroactive_polymer), dated prior to the provisional application filing date.  
 Evaporation (deposition), Wikipedia, [https://en.wikipedia.org/wiki/Evaporation\\_\(deposition\)](https://en.wikipedia.org/wiki/Evaporation_(deposition)), dated prior to the provisional application filing date.  
 Passivation (chemistry), Wikipedia, [https://en.wikipedia.org/wiki/Passivation\\_\(chemistry\)](https://en.wikipedia.org/wiki/Passivation_(chemistry)), dated prior to the provisional application filing date.  
 Physical vapor deposition, Wikipedia, [https://en.wikipedia.org/wiki/Physical\\_vapor\\_deposition](https://en.wikipedia.org/wiki/Physical_vapor_deposition), dated prior to the provisional application filing date.  
 What is Thin Film Deposition by Thermal Evaporation?, Semicore Equipment, Inc., 2020, <http://www.semicore.com/news/71-thin-film-deposition-thermal-evaporation>.  
 Weighing the Benefits of Sputtering v. Evaporation, Denton Vacuum, 2020, <https://www.dentonvacuum.com/weighing-the-benefits-of-sputtering-vs-evaporation/>.  
 International Search Report and Written Opinion of the International Searching Authority for PCT/US21/44566, mailed Nov. 10, 2021.

\* cited by examiner



FIG. 1



FIG. 2

# 1

## PASSIVATED FUEL

### CROSS REFERENCE TO RELATED APPLICATION

This application claims the benefit of U.S. provisional patent application Ser. No. 63/061,377, which was filed on Aug. 5, 2020, and entitled "Passivated Metal Fuel."

### TECHNICAL FIELD

The present invention relates to ignitable metal fuels. More specifically, a non-self-passivating fuel having self-passivating metal fuel layers between the non-self-passivating metal fuel and oxygen source layers is provided.

### BACKGROUND INFORMATION

Various fuel and oxidizer combinations have been known, but in some instances are limited by the reactivity of the fuels. Aluminum is a commonly used metal fuel, partly due to its self-passivating nature. Aluminum will typically form a thin oxide layer on its surface, and will discontinue oxidizing once this passivation layer is formed. However, other desirable metal fuels, for example, magnesium and boron, are prone to self-oxidizing when placed in contact with a source of oxygen or an oxidizer, and are not self-passivating. Instead, magnesium and boron may continue to oxidize until a non-trivial or perhaps substantial portion of the magnesium or boron which is present has been oxidized. For example, magnesium will oxidize to a thickness of about 4 nm when exposed to dry room temperature air, but can oxidize to as much as 50 nm thick or more when exposed to elevated temperatures or humidity.

Some presently known metal fuels rely on the inherent oxidation of the fuel itself, which forms a metal oxide layer on their surface during or after deposition, to passivate the fuel, thereby resisting further oxidation of the fuel. One example is U.S. Pat. No. 5,266,132, which was issued to W. C. Danen et al. on Nov. 30, 1993. Such metal oxide interface layers contribute nothing to the ignition reaction. Their presence within the overall fuel structure combined with their lack of participation in the ignition reaction reduces the energy density of the fuel. When particularly thin fuel layers are used, the formation of these oxide surface layers could potentially consume a significant percentage of the available fuel, making the oxidized fuel unavailable for ignition and considerably reducing the energy density of the fuel. Thus, reliance on the formation of an oxide at the interface between a metal fuel and an oxidizer not only limits the choice of fuels to self-passivating fuels, but also places a minimum limit on the thickness of the fuel layers. Given equal amounts of fuel and oxidizer, a greater number of thinner layers results in faster ignition. However, to the extent that the fuel is oxidized prior to ignition, the oxidized fuel is unavailable for the ignition reaction. Thinner layers of fuel result in oxidation of a greater portion of the fuel, reducing the energy density of the ignition reaction. Thus, fuel selection is limited to those which will self-passivate before a significant amount of the fuel becomes oxidized.

FIG. 1 illustrates the relationship between the fuel size and the lost volume due to oxidation. As this figure demonstrates, a smaller fuel size, such as thinner layers of fuel, result in a greater percentage of that fuel being lost to oxidation during or after deposition of the fuel and oxide layers.

# 2

Deposition techniques which resist the formation of oxide at the interface between a fuel layer and oxide layer include U.S. Pat. No. 8,298,358, issued to Kevin R. Coffey et al. on Oct. 30, 2012, and U.S. Pat. No. 8,465,608, issued to Kevin R. Coffey et al. on Jun. 18, 2013, and the entire disclosure of both patents is expressly incorporated herein by reference. These techniques rely on sputtering chamber pressures of  $10^{-8}$  Torr or perhaps  $6 \times 10^{-9}$  Torr. When such chamber pressures are attainable, these methods have been shown to produce excellent results. Many typical production systems maintain a pressure of  $10^{-5}$  or  $10^{-6}$  Torr, so other means of resisting oxidation of the fuel are desirable when limited to such systems.

Accordingly, there is a need for a self-passivating metal fuel layer that resists oxidation of a non-self-passivating fuel without reducing the energy density of the overall fuel structure. A self-passivating metal fuel layer which could potentially be available itself as fuel would protect the primary, non-self-passivating fuel without causing an appreciable effect on the energy density of the fuel.

### SUMMARY

The above needs are met by a fuel. The fuel comprises a non-self-passivating fuel and an oxygen source. The fuel further comprises a self-passivating metal fuel disposed between the non-self-passivating fuel and the oxygen source.

These and other aspects of the invention will become more apparent through the following description and drawings.

### BRIEF DESCRIPTION OF THE DRAWINGS

FIG. 1 is a graph showing the relationship between fuel size and volume lost due to surface oxidation, comparing a sphere, rod, and sheet.

FIG. 2 is a cross sectional side elevational view of a passivated fuel structure.

Like reference characters denote like elements throughout the drawings.

### DETAILED DESCRIPTION

Referring to FIG. 2, a fuel 10 which includes a passivated fuel is illustrated. The fuel 10 includes one or more non-self-passivating fuel layers 12 and one or more oxygen source layers 14. Each of the fuel layers 12 includes a self-passivating fuel layer 16 disposed on either side of the non-passivating fuel layer 12. As used herein, a self-passivating fuel layer is defined as a layer of material which, when in contact with an oxygen source layer, will react with the oxygen from the oxygen source layer to form an oxide, and will discontinue forming the oxide before the self-passivating fuel layer is completely oxidized, thereby protecting the non-self-passivating fuel layer from oxidation from the oxygen source layer. The portion of the non-self-passivating fuel layer which remains unoxidized remains available as fuel for an ignition reaction with the oxidation layer. Unlike a simple insulating layer, a self-passivating fuel layer thus contributes to the reaction between the non-self-passivating fuel layer and oxide layer by serving as fuel, rather than simply insulating the non-self-passivating fuel layer from the oxygen source layer. An oxygen source layer can be an oxidizer layer such as a metal oxide, or another oxygen source such as a polymer or a single base (nitrocellulose) or double base (nitrocellulose and nitroglyc-

erin) smokeless propellant. In some examples, self-passivating metal fuel **16** is deposited on a polymer **14** substrate such as nitrocellulose, a combination of nitrocellulose and nitroglycerin, or another polymer, followed by a non-passivating fuel **12** and another self-passivating fuel layer **16**. Although a layered structure is illustrated in FIG. 2, as used herein, a layered structure may include a single layer of non-passivating fuel **12** as well as a single layer of an oxygen source **14**, regardless of whether the single layer of oxygen source **14** forms a substrate or a deposited layer.

Each of the fuel layers **12** is a non-self-passivating fuel, for example, magnesium or boron. In the illustrated example, each of the non-self-passivating fuel layers **12** has a thickness ranging from about 10 nm thick to about 50 nm thick, although larger or smaller thicknesses may be used depending on the specific fuel and oxygen source materials selected as well as the desired reaction rate. In the illustrated example, each of the oxygen source layers **14** is shown having a thickness that is similar to the thickness of the non-self-passivating fuel layers **12**. The exact thicknesses of the non-self-passivating fuel layers **12** and oxygen source layers **14**, both in absolute terms and relative to each other, will depend on the amount of fuel and oxygen source that are necessary to substantially fully utilize both the fuel and the oxygen source, and will vary depending on the materials selected. In the illustrated example, the oxygen source layers **14** may be a metal oxide, for example, CuO. Alternatively, the oxygen source layer **14** may be a polymer that is capable of supplying oxygen for the ignition of the fuel layer **12**. Some examples of the layer **14** may be made from a dielectric polymer. A polymer layer **14** could also be selected to introduce nitrogen during ignition, thus lowering the flame temperature.

Other examples of oxygen source layer **14** could be made from nitrocellulose, or a combination of nitrocellulose and nitroglycerin, for example, any such combination used for double base smokeless gunpowder. Each of these materials will burn on its own when ignited, and will also react with the non-passivated metal fuel layer **12** when ignited. In the example of a single base propellant, magnesium will react with nitrocellulose as follows:



Thus, an example combination of magnesium and single base propellant, disregarding the polymer and the protective coating **6**, should consist of about 10.9% magnesium and 89.1% nitrocellulose, +/-2% (excluding the self-passivating layer **16**).

In the example of a double base propellant, disregarding the polymer, magnesium will react with nitrocellulose as shown above, and will react with nitroglycerin as follows:



Thus, an example combination of magnesium and double base propellant, based on a double base propellant having about 40% nitroglycerin, would include about 13% magnesium, 52% nitrocellulose, and 35% nitroglycerin (excluding the self-passivating layer **16**). Double base propellants having different proportions of nitrocellulose and nitroglycerin may be used, with the percentages of nitrocellulose, nitroglycerin, and magnesium varying accordingly. Other burnable metals, for example, boron, will react similarly during ignition of the propellant, so the portions of ingredients for other variations of the propellant, such as those using boron, can be similarly determined.

The layers **16** are made from a self-passivating metal fuel. The illustrated example of the self-passivating fuel layers **16**

are made from aluminum or titanium. In the illustrated example, the self-passivating fuel layers **16** are about 2 nm to about 5 nm thick, although larger or smaller thicknesses could be used. Because aluminum and titanium are self-passivating, the passivation layers **16** will oxidize to the point of self-passivation, and then resist further oxidation, thereby protecting the non-self-passivating fuel layers **12** from oxidation prior to ignition of the fuel structure **10**. Any aluminum or titanium that remains unoxidized remains available as fuel, and will react with the oxygen source layer **14** during an ignition reaction.

As one example, in the case of an oxygen source layer **14** made from CuO and fuel layer **12** made from Mg, the chemical reaction is  $\text{CuO} + \text{Mg} \rightarrow \text{Cu} + \text{MgO} + \text{heat}$ . The reaction therefore requires one mole of CuO, weighing 79.5454 grams/mole, for every one mole of Mg, weighing 24.305 grams/mole. CuO has a density of 6.315 g/cm<sup>3</sup>, and magnesium has a density of 1.74 g/cm<sup>3</sup>. Therefore, the volume of CuO required for every mole is 12.596 cm<sup>3</sup>. Similarly, the volume of Mg required for every mole is 13.968 cm<sup>3</sup>. Therefore, within the illustrated example, each oxygen source layer **14** is about the same thickness or slightly thinner than the corresponding fuel layer **12**. If aluminum is used for the passivation layer **16**, then a small amount of excess CuO can be provided to react with the un-oxidized portion of the aluminum. The amount of excess CuO is determined by the amount of excess aluminum expected to be present to react with CuO according to  $3\text{CuO} + 2\text{Al} \rightarrow 3\text{Cu} + \text{Al}_2\text{O}_3 + \text{heat}$ . If other oxygen sources and fuels are selected, then the relative thickness of the oxygen source layer **14** and fuel layer **12** can be similarly determined.

The layers **12**, **16**, and possibly **14** (depending on the oxygen source selected) can be deposited using the methods described within U.S. Pat. No. 8,298,358, issued to Kevin R. Coffey et al. on Oct. 30, 2012, and U.S. Pat. No. 8,465,608, issued to Kevin R. Coffey et al. on Jun. 18, 2013, and the entire disclosure of both patents is expressly incorporated herein by reference. Dr. Coffey's methods permit the non-self-passivating fuel layers as well as the self-passivating fuel layers deposited using those methods to be either substantially free of oxide (not having a measurable amount of oxide), or if metal oxides of the fuel are present, then the metal oxide layer formed from the fuel will have a thickness of less than about 2 nm or less than about 1 nm.

The layers **12**, **14**, and/or **16** may also be deposited using sputtering, evaporative deposition, physical vapor deposition, or chemical vapor deposition. The presence of the self-passivating layer **16** between the non-self-passivating fuel **12** and oxygen source **14** makes oxidation of a portion of the self-passivating fuel layer **16** acceptable, and ensures that the primary fuel, found in the non-self-passivating layer **12**, is protected from oxidation. In some examples, a fuel layer **12** may be deposited on a self-passivating layer **16** that has been deposited on a polymer sheet **14**, for example, a nitrocellulose sheet **14** or a sheet **14** made from nitrocellulose and nitroglycerin.

During or after deposition, a portion **18** of the layer **16** which is adjacent to the oxygen source layer **14** may oxidize. Because the material and the thickness of the layer **16** are selected to ensure that the layer **16** will self-passivate prior to the oxidation reaching the fuel layer **12**, an unoxidized portion **20** of the layer **16** will remain. This unoxidized portion **20** is available as fuel for an ignition reaction.

As an alternative to a layered fuel structure, other fuel structures may be used. For example, a fuel utilizing granules or pellets of fuel and oxygen source may utilize fuel pellets made from non-self-passivating fuel that is substan-

tially covered by self-passivating fuel. As used herein, substantially covered means that the non-self-passivating fuel is sufficiently covered to resist oxidation by the oxygen source prior to ignition of the fuel.

While not limited to such use, the fuel structure 10 described herein is anticipated to be useful as a propellant or as a payload for munitions, including but not limited to small arms, artillery, and rockets. The fuel 10 can be utilized for applications where high explosives can otherwise be used. The fuel structure is also anticipated to be useful as a primer for firearms and other munitions which use a primer. As another alternative, multiple ignition or detonation points utilizing controlled timing of ignition or detonation may be incorporated into the fuel 10. Specific ignition/detonation timing and control structures and methods are disclosed in U.S. Pat. No. 9,464,874, which was issued to Timothy Mohler et al. on Oct. 11, 2016, U.S. Pat. No. 9,709,366, which was issued to Timothy Mohler et al. on Jul. 18, 2017, U.S. Pat. No. 9,816,792, which was issued to Timothy Mohler et al. on Nov. 14, 2017, and U.S. Pat. No. 10,254,090, which was issued to Timothy Mohler et al. on Apr. 9, 2019. The entire disclosure of each and every one of these patents is expressly incorporated herein by reference.

The present invention therefore provides a fuel structure that can utilize the advantages of non-self-passivating fuels such as magnesium or boron, while resisting oxidation of those fuels through contact with an adjacent oxygen source. Additionally, the passivation layer itself may also serve as fuel for the ignition reaction.

A variety of modifications to the above-described embodiments will be apparent to those skilled in the art from this disclosure. Thus, the invention may be embodied in other specific forms without departing from the spirit or essential attributes thereof. The particular embodiments disclosed are meant to be illustrative only and not limiting as to the scope of the invention. The appended claims, rather than to the foregoing specification, should be referenced to indicate the scope of the invention.

What is claimed is:

1. A fuel, comprising:  
a non-self-passivating metal fuel;  
an oxygen source; and  
a self-passivating metal fuel disposed between the non-self-passivating metal fuel and the oxygen source;  
whereby the self-passivating fuel oxidizes by reacting with the oxygen source to form a passivation layer, the passivation layer resisting oxidation of the non-self-passivating fuel from the oxygen source until the fuel is ignited.
2. The fuel according to claim 1, wherein:  
the fuel has a layered structure;  
the non-self-passivating fuel forms at least one layer of the layered structure, the at least one layer of non-self-passivating fuel defining a pair of opposing surfaces;  
the oxygen source forms at least one layer of the layered structure; and  
the self-passivating metal fuel is disposed on each of the opposing surfaces of the non-self-passivating fuel.
3. The fuel according to claim 2, wherein the non-self-passivating metal fuel is boron or magnesium.
4. The fuel according to claim 3, wherein the oxygen source is a metal oxide, a polymer, or a combination thereof.
5. The fuel according to claim 4, wherein the self-passivating metal fuel is aluminum or titanium.
6. The fuel according to claim 1, wherein the non-self-passivating metal fuel is boron or magnesium.
7. The fuel according to claim 6, wherein the oxygen source is a metal oxide, a polymer, or a combination thereof.
8. The fuel according to claim 7, wherein the self-passivating metal fuel is aluminum or titanium.
9. The fuel according to claim 1, wherein the oxygen source is a metal oxide, a polymer, or a combination thereof.
10. The fuel according to claim 1, wherein the self-passivating metal fuel is aluminum or titanium.
11. The fuel according to claim 1, wherein the self-passivating metal fuel substantially covers the non-self-passivating metal fuel.

\* \* \* \* \*